

## UNITED STATES PATENT OFFICE

2,518,153

## DYEING OF CELLULOSE ESTERS WITH REDUCED VAT DYES IN ALCOHOLIC SOLUTION

Edwin R. Laughlin, West Newton, Mass., and Raymond W. Foulk, Bridgeport, N. J., assignors to E. I. du Pont de Nemours & Company, Wilmington, Del., a corporation of Delaware

No Drawing. Application January 7, 1948,  
Serial No. 1,066

2 Claims. (Cl. 8—36)

1

This invention relates to the dyeing of cellulose esters, and more particularly to the dyeing of fabrics composed of or containing cellulose esters, such as cellulose acetate, with vat dyes.

Vat dyes are used extensively in the dyeing of cellulose fibers such as cotton, regenerated celluloses, etc., when it is desired to impart to those fibers colors having maximum fastness properties, especially fastness to light, weather and laundering. Because the vat dyes are usually applied to cellulose material from solutions having relatively high alkalinity, they have not found general application in the dyeing of cellulose acetate or other esters because the highly alkaline vat causes saponification of the cellulose ester with the result that the desirable characteristics and advantages which the cellulose acetate fibers possess over the viscose rayons is lost.

Cellulose acetate and other esters are customarily dyed with "acetate colors," which, although they exhibit moderate to fairly good light fastness, do not exhibit the fastness to washing, especially repeated washing or laundering, that is desired, and some of the dyes of this class are sensitive to gas fume fading and undergo drastic changes in color when the dyed material is exposed to fumes of burning natural gas, oxides of nitrogen and other gases normally present in the atmosphere, particularly in highly industrialized communities.

The fact that it has heretofore been impossible to dye cellulose acetate readily in a range of colors which may be characterized as "fast" in the same sense that fast colors are easily obtainable on other textile fibers, such as cotton, regenerated celluloses, silk and wool, has materially retarded the more extensive use of cellulose acetate as a textile material. A continuing effort is being made to provide a commercially feasible process for dyeing cellulose acetate with dyes which have better fastness properties than those that are now available for general use on that fiber, and with a class of colors that permits a wider range of shades.

Previous attempts have been made to dye cellulose acetate with reduced vat dyes from the usual vat employed in the dyeing of cotton and regenerated celluloses, but it has been found that, if the time of dyeing is comparatively short, little or no color is imparted to the fiber, while, if a longer time of contact is employed, the alkaline dye liquor causes saponification of the cellulose ester, resulting in the formation of some cellulose for which the dye liquor has greater substantivity than for the cellulose acetate, thereby causing

2

very uneven and undesirable dyeings. Another proposal has been to replace the strong alkalies normally used in vat dyeings by weak alkalies. However, such a process limits the number of vat dyes applicable and actually does not completely prevent saponification.

It is an object of this invention to provide a process for dyeing cellulose acetate and related esters with vat dyes. A further object of the invention is to provide a commercially feasible process for the dyeing of cellulose acetate with vat dyes without damage to the acetate and without causing any material amount of saponification of the same during the dyeing process. Another object of the invention is to provide a process for dyeing cellulose acetate with all types of vat dyes. A still further object of the invention is to permit vat dyeings of cellulose acetate by a continuous process without saponification so that all the excellent esthetic and physical properties of this valuable fiber are retained. Further objects will appear hereinafter.

We have found that the above objects may be very effectively accomplished by maintaining a relatively high concentration of alcohol in the alkaline hydrosulfite vat of the vat dye together with a wetting agent, a dispersing agent, and an additional type of adjuvant which we call a vat-stabilizing agent consisting of diethylene glycol, thiidiethylene glycol, or glycerine. The cellulose ester absorbs in this manner a sufficient amount of the dye liquor to impart the desired color thereto, and if the alkalinity of the solution in the fiber is quickly lowered to a point where saponification of the fiber does not occur, very satisfactory dyeings with the vat dye can be attained. By this method, we have found that the cellulose ester fiber itself is not harmed or degraded and the dyed material possesses the excellent fastness properties usually associated with this type of dye when applied to cotton or regenerated cellulose.

The alcohol which acts as a swelling agent on the cellulose ester fiber permits the leuco vat dye to quickly penetrate into the fiber itself. For the purpose of our invention we have found that alcohols having up to and including four carbon atoms, such as tertiary-butyl, propyl, isopropyl, ethyl, and methyl alcohols are of particular advantage. Of these alcohols the most effective are propyl, isopropyl and ethyl alcohols. To carry out our invention the alcohol concentration should be maintained between 30% and 60% by volume of the reduced pad bath liquor and the alcohol should be fully miscible with water at the concentration used.

It is necessary to employ in the padding solution agents which will facilitate uniform wetting and swelling of the cellulose esters. In addition the leuco vat color must either be completely in solution or in a state of highly dispersed colloidal solution for successful operation. The use of dispersing agents in aqueous systems has long been used. We find that their use is helpful in our process, but the dispersing agents for use in the aqueous-alcohol media are by themselves not satisfactory when the final alcohol content in the solution is 30% to 60% which is within the scope of our invention. At such concentrations of alcohol the leuco vat color quickly agglomerates and is precipitated. We have found that certain agents which we call vat-stabilizing agents can be used to enable the vat leuco to remain either dissolved or highly dispersed in the presence of such a great quantity of the alcohol. The vat-stabilizing agents which we have found effective are polyhydroxy alkyl compounds such as diethylene glycol, thiadiethylene glycol, or glycerine.

Any of the wetting agents usually employed in the dyeing or treating of textile fibers may be used in this process, such as the sodium salt of the sulfates of straight chain aliphatic alcohols containing eight or more carbon atoms, the sodium salts of the alkyl naphthalene sulfonic acids such as isopropylated naphthalene sulfonic acid, the sodium salts of the sulfonates of higher molecular weight aliphatic hydrocarbons, the sodium salts of sulfonated tetralin, etc.

The dispersing agents may be any of those suitable for dispersing finely divided solids in alkaline solutions, such as sodium ligno-sulfonates, the naphthalene beta-sulfonic acid formaldehyde condensation products such as produced by the process of United States Patent 1,836,759, the triamine bases such as the trialkyl trimethylene triamines, etc.

The wetting agent is preferably employed in the dye bath in an amount ranging from 0.1 to 4 ounces per gallon. The dispersing agent and the glycerine or glycols may each be used in an amount ranging from 0.25 to 4 ounces per gallon of dye solution.

In practice, the material to be dyed may be padded in the alkaline hydrosulfite vat of the vat dye containing the alcohol, the swelling agent, the dispersing agent, and the vat-stabilizing agent. The fabric is then passed immediately into a bath of lower alkalinity such as water, or, preferably, a soda ash development bath of the type described in United States Patent 2,318,133. The cellulose ester is then rinsed, the dye oxidized, and the material dried.

For satisfactory operation as a continuous process it is necessary that the temperature be sufficiently high to insure prompt swelling of the cellulose ester, but not so high that saponification of the fiber occurs in any substantial amount, or that much of the alcohol is lost by vaporization. We have found that in the padding operation temperatures in the range of 110° F. to 150° F. are operable, but the preferred range is 115° F. to 140° F. Below 110° F. swelling of the fiber is slow, while above 150° F. saponification takes place. The time in the pad-bath must be sufficient to allow good swelling, but not so great that saponification of the fabric commences. The immersion time depends on the alcohol used, the alcohol concentration and the temperature of

the pad-bath. For the purpose of our invention this time may range generally from four to ten seconds.

After padding through the aqueous alcohol solution, the fabric is squeezed sufficiently to prevent "run-back" of color on the fabric as it is carried over and under the guide rolls. We have found that with cellulose acetate the liquor retention by the fabric, or "pick-up" as it is called in the trade, should be in the range of 40% to 100%, based on the weight of the cloth, but the preferred range is 50% to 70%.

The following examples are given to illustrate the invention. In these examples the ingredients added are based on ounces by weight per gallon of dye solution.

#### Example 1

A two ounce per gallon pad liquor of "Ponsol" Golden Orange RRT (Color Index 1098) was prepared as follows:

2.0 oz. "Ponsol" Golden Orange RRT paste (11% color solids)  
 25 2.0 oz. potassium hydroxide  
 2.5 oz. sodium hydrosulfite  
 2.0 oz. sodium hydrocarbon sulfonate wetting agent (product of Example III of U. S. P. 2,366,027)  
 30 1.0 oz. naphthalene sulfonic acid-formaldehyde condensation product  
 2.5 oz. diethylene glycol

Reduction was carried out for 15 minutes at 140° F. in 3.5 pints of water. The volume was made up to 0.5 gallon with water and then 0.5 gallon of ethyl alcohol and 0.5 oz. of triethyl trimethylene triamine were added. Cellulose acetate satin was padded with this liquor at 120° F. for six seconds and at 55% "pick-up," and was then immediately led into an aqueous soda ash development bath for 60 seconds at 120° F. which contained:

45 1.00 oz./gal. soda ash  
 0.08 oz./gal. potassium hydroxide  
 0.25 oz./gal. sodium hydrosulfite  
 4.00 oz./gal. common salt

The fabric was then oxidized by passing through a bath containing:

0.13 oz./gal. sodium dichromate  
 0.40 oz./gal. acetic acid 28%

Following this, the fabric was rinsed, soaped, rinsed, and dried.

The resultant fabric was uniformly dyed a pleasing reddish-orange of excellent fastness to light, crocking, perspiration and repeated laundering. Furthermore, the resultant fabric had not been damaged nor saponified. The class of dyes known as direct dyes will dye viscose rayon readily and leave cellulose acetate unstained. The most sensitive indication of saponification of cellulose acetate consists in subjecting the material to the action of a direct dye bath. If even a trace of surface saponification has occurred, too small to be determined by the customary acetone solubility or hydrolysis tests, the material will nevertheless be stained by the direct dye. In the above example, the material was cross-dyed with "Pontamine" Sky Blue 6BX, Color Index 518, and left completely unstained, indicating that there had been no trace of saponification.

## Example 2

A 0.5 ounce per gallon pad liquor of "Ponsol" Golden Orange RRT (Color Index 1098) was prepared as follows:

5      0.5 oz. "Ponsol" Golden Orange RRT paste (11% color solids)  
 1.5 oz. potassium hydroxide  
 1.8 oz. sodium hydrosulfite  
 2.0 oz. sodium hydrocarbon sulfonate wetting agent (product of Example III of U. S. P. 2,366,027)  
 1.0 oz. naphthalene sulfonic acid-formaldehyde condensation product  
 2.5 oz. diethylene glycol

Reduction was carried out for 15 minutes at 140° F. in 3.5 pints of water. The volume was made up to 0.5 gallon of water, and then 0.5 gallon of ethyl alcohol and 0.5 oz. of triethyl trimethylene triamine were added.

The dyeing of the cellulose acetate satin was carried out as in Example 1 to give equally satisfactory results.

## Example 3

A four ounce per gallon pad liquor of "Ponsol" Golden Orange RRT (Color Index 1098) was prepared as follows:

25      4.0 oz. "Ponsol" Golden Orange RRT paste (11% color solids)  
 2.0 oz. potassium hydroxide  
 2.5 oz. sodium hydrosulfite  
 2.0 oz. sodium hydrocarbon sulfate wetting agent (product of Example III of U. S. P. 2,366,027)  
 1.0 oz. naphthalene sulfonic acid-formaldehyde condensation product  
 2.5 oz. diethylene glycol

Alkaline reduction was carried out for 15 minutes at 140° F. in 3.5 pints of water. The volume was made up to 0.5 gallon of water and 0.5 gallon of ethyl alcohol and 0.5 oz. of triethyl trimethylene triamine were added.

The cellulose acetate satin was then dyed and finished in the manner described in Example 1 above to give a dyeing which was equally satisfactory.

Thiodiethylene glycol and glycerine may be substituted in the above Examples 1, 2, and 3 for diethylene glycol and at the same concentration to give equivalent effectiveness as vat-stabilizing agents.

## Example 4

The following vat colors were applied to cellulose acetate satin by the process similar to that described in Examples 1, 2, and 3 with equivalent satisfying results:

Sulfanthrene Yellow R supra..... C. I. #1170  
 Sulfanthrene Orange R paste..... C. I. #1217  
 Vat dye of Example 3 of U. S. P. 1,234,171  
 Sulfanthrene Red 3B paste..... C. I. #1212  
 Sulfanthrene Blue 2BD paste..... C. I. #1184  
 Sulfanthrene Blue GR paste..... C. I. # 969  
 Sulfanthrene Navy Blue MR paste..... C. I. #1183  
 Vat dye of Example 1 of U. S. P. 1,090,621  
 Ponsol Yellow G double paste..... C. I. #1118  
 Ponsol Yellow AR double paste..... C. I. #1132  
 Ponsol Golden Orange G paste..... C. I. #1096  
 Ponsol Brown AG double paste..... C. I. #1152  
 Ponsol Brown AR double paste..... C. I. #1151  
 Ponsol Brown BB paste..... C. I. #1120  
 Vat dye of Example 3 of U. S. P. 1,329,435  
 Ponsol Red BN double paste..... C. I. #1162  
 Ponsol Violet AR double paste..... C. I. #1135  
 Ponsol Brilliant Violet 3B paste..... C. I. #1105

Ponsol Violet 2RD paste..... C. I. #1104  
 Ponsol Red Violet RRNX paste..... C. I. #1161  
 Ponsol Blue BF double paste..... C. I. #1113  
 Ponsol Blue GD double paste..... C. I. #1112  
 Ponsol Blue BCS double paste..... C. I. #1114  
 Ponsol Brilliant Blue R paste..... C. I. #1106  
 Ponsol Blue 3G paste..... C. I. #1109  
 Vat dye of Example 1 of U. S. P. 1,761,624  
 Ponsol Dark Blue BR paste..... C. I. #1099  
 Ponsol Jade Green double paste..... C. I. #1101  
 Vat dye of Example 2 of U. S. P. 1,596,528  
 Ponsol Olive AR double paste..... C. I. #1150  
 Vat dye of U. S. P. 995,396  
 Ponsol Black BA double paste..... C. I. #1102

15      The advantages of our invention are obvious. We are enabled to dye cellulose ester fabrics with the full range of vat colors without the attendant disadvantages of saponification of the fiber. The result leads to a cellulose ester fabric dyed with the fastest line of dyestuffs known today. The vat colors also may be applied in fairly heavy shades, and the deficiencies of poor fastness to light, rubbing, perspiration, washing, especially repeated washing and laundering and gas fume fading are overcome by our process. An especial advantage is the fact that the cellulose ester fabric after vat dyeing by our process shows no adverse effects or deterioration but fully retains all of the esthetic properties of pleasing handle and outstanding draping qualities inherent in this type of fabric. A further advantage of our invention is that due to the rapidity with which the process may be performed it is readily applicable to continuous process.

We claim:

1. A process of dyeing cellulose esters with vat dyes, which comprises padding the cellulose ester material for a period no more than 10 seconds with an aqueous alkaline solution of a reduced vat dye containing in the solution from 30% to 60% of alcohol, and, for each gallon of dye liquor, alkali in an amount equivalent to no more than 2.0 ounces of potassium hydroxide, from 0.1 to 4 ounces of a wetting agent, 0.25 to 4 ounces of a dispersing agent and from 0.25 to 4 ounces of a stabilizing agent of the group consisting of diethylene glycol, thioldiethylene glycol and glycerine, maintaining the pad bath temperature between 110° F. and 150° F. and, immediately after padding, passing the material into an aqueous solution having an alkalinity below that at which saponification of the cellulose ester takes place, and oxidizing the reduced vat dye on the material.

2. In a continuous process for dyeing cellulose acetate fibers, the steps which comprise padding the fibers for a period no more than 10 seconds with an aqueous alkaline solution of the reduced vat dye containing in the solution from 30% to 60% of alcohol, and, for each gallon of dye liquor, alkali in an amount equivalent to no more than 2.0 ounces of potassium hydroxide, from 0.1 to 4 ounces of a wetting agent, 0.25 to 4 ounces of a dispersing agent and from 0.25 to 4 ounces of a stabilizing agent of the group consisting of diethylene glycol, thioldiethylene glycol and glycerine, maintaining the pad bath temperature between 110° F. and 150° F. and, immediately after padding, passing the impregnated fibers into a solution having an alkalinity below that at which saponification of the cellulose acetate takes place, and thereafter oxidizing the reduced vat dye on the fiber.

EDWIN R. LAUGHLIN.  
 RAYMOND W. FOULK.

(References on following page)

## REFERENCES CITED

The following references are of record in the file of this patent:

## UNITED STATES PATENTS

| Number    | Name     | Date          |
|-----------|----------|---------------|
| 1,398,357 | Briggs   | Nov. 29, 1921 |
| 1,968,856 | Rivat    | Aug. 7, 1934  |
| 2,067,926 | Kern     | Jan. 19, 1937 |
| 2,090,511 | Crossley | Aug. 17, 1937 |

## FOREIGN PATENTS

| Number  | Country       | Date          |
|---------|---------------|---------------|
| 479,867 | Great Britain | Feb. 14, 1938 |
| 847,107 | France        | June 26, 1939 |
| 583,349 | Great Britain | Dec. 16, 1946 |

## OTHER REFERENCES

Amer. Dye. Rep. for May 21, 1945, page P212.  
Rayon Textile Monthly for March 1947, page 100 (158).